

Jan. 12, 1965

R. J. SCHMIDT

3,165,036

PAVING STRUCTURE

Filed March 1, 1963



FIG. 1



FIG. 2



FIG. 3

INVENTOR  
ROBERT J. SCHMIDT  
BY C. L. Snow  
D. F. Rocq  
ATTORNEYS

**1**

3,165,036

**PAVING STRUCTURE**

Robert J. Schmidt, El Cerrito, Calif., assignor to California Research Corporation, San Francisco, Calif., a corporation of Delaware

Filed Mar. 1, 1963, Ser. No. 263,377

14 Claims. (Cl. 94—7)

The present invention relates to composite-type pavement structures and method of preparing the same, and particularly to such structures which can be applied as overlays for strengthening, resurfacing, and protecting various pavements and road surfaces. More particularly yet, it relates to laminated overlays serving to reinforce pavements subjected to extensive wear due to heavy traffic, to minimize skidding, to provide a warning to motorists approaching dangerous portions of a road, such as curves and intersections, and to protect pavements from damage which may be occasioned by water and spilled solvents and liquids.

It has been suggested already to employ plastic overlays to reinforce and to protect Portland cement concrete (PCC), asphalt-concrete (AC), and other like pavements apt to become damaged by cracking under the continued impact of intensive daily traffic load, this cracking being aggravated by the adverse action of water and atmospheric moisture and by spillage of oil, grease and motor fuels.

Accordingly, various plastic materials, e.g., alkyd resins, epoxy resins and asphalt, have been applied as seal coats or overlays on different pavement surfaces whenever the particular circumstances seemed to justify their use. For instance, to reduce the risk of skidding of motor vehicles on curves and at intersections, particularly in wet weather, plastic overlays, specifically asphalt overlays, containing sand and/or other suitable, comparatively fine, particulate solid materials have been applied onto the pavement. Plastic overlays, colored to attract attention and to give a visual warning to the approaching motorist, have also been tried in various locations.

Likewise, "rumble strips" in the form of pavement overlays prepared with asphalt and placed in sequence across a traffic lane and in which large aggregate is bonded in the plastic to form a jagged, sawtooth-like surface, have been proposed to give an audible warning to slow down to motorists approaching a hazard by giving rise to a higher noise level and by vibrating the vehicles.

Plastic overlays have also been considered and employed as seal coats on pavements built of Portland cement concrete (PCC) and asphalt-concrete (AC) to minimize the damage likely to be suffered by the pavement surface from the adverse action of oil, grease, and fuel. However, the actual experience has pointed out that not every plastic material can be employed satisfactorily as a pavement overlay, although such an overlay may appear initially to be an effective anti-skid coating, a rumble strip or a seal coat.

Asphalts which have been proposed for use in such overlays lack strength, tend to soften up and to melt in warm weather with loss of aggregate, and, upon expansion and contraction with the change of ambient tem-

**2**

perature, form little cracks and crevices through which water penetrates and then freezes at lower temperatures, damaging the underlying road base. Furthermore, asphalts are not impervious to petroleum fluids, such as oil and gasoline.

Many of the synthetic thermoplastic resins, although easily applied to the pavement surface, lack satisfactory adhesion and tend to flow and to deform under load and, are very vulnerable to attack by solvents.

- 10 Thermosetting resins, owing to their high tensile, flexural, impact and adhesion strengths, high distortion temperatures and softening points, resistance to water, hydrocarbons, etc., as a general rule, produce good surface cover (overlays) for Portland cement concrete, asphalt-concrete, and other rigid-base pavements. However, their acceptance by the trade has been hindered so far by several serious drawbacks attendant to their utilization, namely, necessity of a special preparation of the underlying surface before applying the resin, precise control 15 and timing of its application, and, particularly, eventual occurrence of cracks in the underlying pavement upon setting, due to the differences between the coefficient of expansion of the thermosetting resin and that of the underlying pavement base, particularly if this base is formed by asphalt-concrete. The resin, once it has set, forms a very strong bond with the underlying pavement which will not yield when subjected to thermal stresses. The result is cracking and eventual disintegration of the base, since ground water and rain water seep through the cracks, 20 and, upon alternate freezing and thawing, further promote the breaking of the pavement.

The present invention is directed at enabling successful utilization of thermosetting resins in pavement overlays, wherein the resin is present as one or as several 25 layers of a laminated paving structure and in which the aforementioned tendency toward cracking and deterioration is substantially eliminated. This is achieved by the introduction of a layer of a thermoplastic bituminous material, such as an asphalt, between the underlying pavement and the surface coating of the resin. In the laminated pavement structure thus constructed, when this 30 structure is subjected to the conditions of thermal stress, such as occur during the cure of the overlay and with subsequent variations of ambient temperature, the layer 35 of bituminous material acts as a slip-plane and the rigid resin surface moves independently of the pavement structure below. Therefore, the underlying pavement does not crack and does not allow water to penetrate there-through, while the resin layer minimizes the likelihood 40 of injury to the pavement by contact with other solvents that may be spilled on the top surface of the overlay.

In its simplest form, the laminated pavement structure of the invention can be represented as shown in FIG. 1 of the drawing attached to this specification. In 45 FIG. 1, A is the pavement base of an asphalt-concrete, Portland cement concrete, or the like. B is a layer of asphalt acting as the slip-plane and applied onto A either as hot liquid asphalt or as an emulsion of asphalt in water. This layer B is followed by a layer C consisting of mineral aggregate, such as stone, stone chips, gravel or sand, to provide an adequate barrier between the asphalt layer B and the layer of resin D which is applied next onto the aggregate layer C, for instance, by

spraying. This barrier is desirable because an unduly long direct contact with asphalt during the resin cure may interfere with the setting (hardening) of certain thermosetting resins. As a matter of fact, such a barrier will be interposed between the top thermosetting resin layer and the slip-plane layer of any thermoplastic bituminous material, soluble in carbon disulfide and containing free-radical inhibitors, and, consequently, apt to inhibit the cure of thermosetting resins which set (harden) by a free radical mechanism, as typified by the hardening of unsaturated polyester resins. The thermoplastic materials which, by virtue of their bituminous character and their content of free-radical inhibitors, particularly tend to inhibit the resin cure, are various asphalts, pitches and tars, adequately rigid at normal temperatures and under normal conditions of stress, but otherwise capable of deformation when subjected to heat and pressure. The asphalts may be steam-refined, solvent-refined, air-blown, and the like, and they may be used either as such or blended in a suitable manner with "native" bitumens, such as gilsonite. The tars which are effective in "slip-planes" of the paving structures of the present invention may be, for instance, coaltars from gasworks retorts, coke ovens, blast furnaces, etc. The pitches are those obtained from the distillation of various tars. The thermosetting resin may be any thermosetting resin hardening by a free radical mechanism, for instance, a phthalic acid polyester resin which, upon being sprayed, penetrates and binds together the aggregate surface. Preferably, in order to prevent slipperiness and to impart a particular desired characteristic to the resin surface, it is topped by a layer of a finely particulate solid, such as sand, sawdust, cut colored fibers, coloring-sand mixtures, etc. as shown by E in FIG. 1.

Also, several successive layers of resin or alternating layers of resin and sand may be employed, depending on the ultimately intended use of the overlay, whether as a seal coat on a road, on a runway of an airport, on the surface of a wharf, or a bridge, and the like.

One advantage of applying these overlays is that no complicated precleaning of the original pavement surface is required. In other words, no necessity exists for resorting to a sequence of sweeping, steam cleaning, and, finally, etching the surface with dilute alkali or acid. It suffices to sweep the pavement surface, whether concrete (PCC) or asphalt-concrete (AC), of all loose material, whereupon the asphalt layer may be immediately applied thereto either as a hot asphalt or as an asphalt emulsion (anionic or cationic). The stone aggregate is applied immediately thereafter. If asphalt has been applied as an emulsion, the application of resin is postponed until the emulsion is sufficiently dehydrated. Otherwise, the resin may be immediately sprayed on the surface of the aggregate.

For certain specialized applications of these overlays, such as "rumble strips," and "armor coats," an intermediate "choke layer" of sand or other suitable finer aggregate, will precede the application of resin. The resin is then applied in a sufficient amount to bind firmly the surface of the "choke" (sand fill) and any protruding coarser aggregate surfaces by one continuous coating. Thereafter, a final application of a finely particulate solid material, such as sand, cut fibers, saw dust, iron oxide, etc. will produce the desired outside surface. Before opening the road to traffic, excess of sand or like topping material is simply swept off. In general, the asphalt is applied at a rate of about 0.1 to 0.5 gallon per square yard of the paved surface; for coarse-textured overlay structures rates from about 0.25 to about 0.5 gallon of asphalt per square yard are preferred. On Portland cement concrete and in overlays prepared with finer aggregates, generally less asphalt will be employed. These rate figures refer to undiluted asphalt, and in the

case of asphalt emulsions, the rate is based on the actual asphalt content thereof. Any suitable mineral aggregate conventionally used for paving work may be employed in the preparation of the overlays in accordance with the invention. The size of the individual particles (stones) of the aggregate, their nature and texture are not critical and are chosen in accordance with the local conditions and requirements of each particular case. However, in the construction of "rumble strips," which will be described later on, the aggregate to be embedded in the asphalt atop the underlying pavement base generally varies in size from  $1\frac{1}{2}$ " to  $\frac{3}{8}$ ", meaning that the majority of the stones in such aggregate has linear dimensions lying between these limits. Accordingly, in such cases, the "choke layer" is formed by an aggregate which is finer in size than the first embedded aggregate.

A particular embodiment of the invention relates to the preparation of the so-called "rumble strips." They are placed atop a pavement in locations adjacent to dangerous intersections and curves, so that the tires of and, consequently, the motor vehicle itself in riding over these strips become subjected to a greater degree of vibration than in riding over the regular pavement surface of the same road. This vibration is translated both into a tactile and an audible warning as the vehicle approaches the danger, causing the driver to slow down.

A schematic representation of such "rumble strip" overlay paving structure is shown in FIG. 2 of the drawing. In FIG. 2, the numeral 1 designates the underlying pavement base. A layer of asphalt 2 is applied at the rate from approximately 0.10 to about 0.50 gallon per square yard onto this base surface. The rate figures are based on undiluted asphalt so that, if an asphalt emulsion (anionic or cationic) is employed, the rate figures refer to the actual asphalt content of this emulsion.

A course of coarse stone aggregate, from  $1\frac{1}{2}$ " to  $\frac{3}{8}$ " in size and one stone in thickness, is then embedded into the asphalt which is employed in an amount sufficient to bind these stones but not to submerge them. This stone course is designated 3 in FIG. 2. A "choke layer" of sand or other suitable finer mineral aggregate, designated by 4, is then applied to fill the interstices of the individual stones of layer 3 and to form a more or less impervious barrier between the asphalt and the coating of a thermosetting resin which is applied following the "choking" step. The purpose of the "choke layer" is to forestall the contact of the resin with the asphalt (or any other thermoplastic bituminous material, when it is used in lieu of asphalt). As mentioned before, when this contact is prolonged, it may inhibit the cure of certain thermosetting resins, probably owing to the presence of free-radical inhibitors, such as phenolic constituents in the asphalt. Before spraying on the resin, excess of sand is swept off. The resin is then applied (in one or several successive layers) using any suitable application technique. It binds the individual particles of the "choke layer" and coats the protruding portions of the coarse stone aggregate, forming a continuous rigid surface film 5. To impart the desired non-slippery texture to the outer surface of the rumble strip overlay, sand is applied onto the resin coating before it becomes hardened. Upon setting, the excess sand may be swept off. If desired, several applications of resin and sand, successively or simultaneously, may be applied onto the original resin coating.

The following observations confirmed the necessity of providing, according to the invention, a "choke layer" of finer stone aggregate to separate substantially completely the bituminous thermoplastic "slip-plane" from the layer of polyester resin, when using for this "slip-plane" a tar which tends to inhibit the resin cure.

A coating emulsion of coal tar available on the market under the trademark "Colfix" was employed to coat a 7" x 14" x 2" specimen of asphalt concrete pavement.

When the emulsion has broken (set), a thin layer of a high-impact, flexible polyester resin of the same kind as in the tests described hereinbefore where asphalt was used in the slip-plane, was applied to the tar-coated surface of the specimen. However, after three weeks, the surface was found to have remained tacky, indicating the failure of the resin to cure satisfactorily. Increasing the thickness of the resin layer did not provide a more satisfactory coating. In fact, after three weeks, on being peeled back with a knife, the polyester-coal tar interface was again found to have remained tacky.

On the other hand, when a similar specimen of asphalt concrete pavement coated with the same coal tar emulsion received first an application of one-half inch aggregate and No. 10 mesh sand, and then was given an application of the aforementioned polyester resin, the resin became completely cured within  $1\frac{1}{2}$  hours without any indication of tackiness, bond failure between the resin layer and the concrete base, or cracks in the resin coating. It was evident that the cure of the resin has not been at all inhibited, and that the "choke layer" served as an effective physical barrier separating the coal tar and the resin.

In "armor coat"-type overlays, that is, in overlays which are used to protect portions of road surfaces exposed to heavy traffic loads, the aggregate embedded in the asphalt layer applied onto the original pavement surface need not be as coarse as in the case of "rumble strips." Since in "armor coats" the top surface is to be rather smooth and the aim is not to produce vibration and rumbling noise, aggregate stone sizes from about 1" to about  $\frac{1}{4}$ " are found satisfactory. The quantity and the rate of application of the asphalt correspondingly may also be somewhat lower. For "choking," a suitable aggregate (sand or grits) of a finer size will be used, also followed by a layer (or layers) of thermosetting resin and by a final seal-coat (or coats) of resin and sand. Preferably, several courses of resin and fine aggregate will be applied to produce a firm, non-skid protective overlay.

On the other hand, where a thin, lightweight ( $\frac{1}{4}$ " or less) overlay is desired, whether to provide a solvent-resistant surface and to prevent "raveling" or to reduce the risk of skidding, an even finer stone aggregate, from about  $\frac{3}{8}$ " to about  $\frac{1}{8}$ ", will be embedded in the asphalt layer, the asphalt being applied at a rate from approximately 0.10 to 0.50 gallon per square yard, usually from about 0.10 to 0.15 gallon per square yard.

A schematic representation of an "armor coat" or a lightweight overlay is shown in FIG. 3 of the drawing.

In this figure, the symbol *a* designates the original pavement surface; *b* designates the asphalt slip-plane layer; *c*, designates the coarse aggregate; *d*, the finer aggregate or sand "choke"; *e*, the coating of resin; and *f*, sand or grits held in resin in a firm, fine-textured seal-coat surface.

In all of these different embodiments of laminated overlays of the invention, in accordance with requirements of each particular case, several coats of resin may be successfully applied before the final resin-sand application, or several alternating layers of resin and sand may be employed to protect the underlying pavement structure. In all instances, clean, dry aggregate of more or less the same size should be employed. For better non-skid effect, stones with high polishing resistance or special anti-skid materials, such as crushed granite chips, sharp crushed sand, aluminum oxide, carborundum and the like are to be preferred.

As to the actual practical construction of overlays in accordance with the invention, any suitable and readily available equipment may be employed for the purpose.

The asphalt is applied as any conventional seal coat, and the stone aggregate, particularly when preparing "rumble strips" is embedded by light "pneumatic-tire" rolling, to avoid the risk of grinding or breaking the stones. Fine aggregates, such as chips or sand, are spread

in any suitable effective manner, for instance, from tailgate mobile spreaders.

In applying the resin, where areas to be covered by an overlay are small, the operation may be done by hand; otherwise, any suitable equipment, such as travelling spray-bar or twin spray-bars with multiple heads mounted on a trailer may be employed.

As pointed out before, any thermosetting resin, such as phenolic resins, epoxy resins, unsaturated polyester resins and the like, may be employed. Unsaturated polyester resins prepared by reacting polyhydric alcohols or phenols with polybasic (preferably aromatic) acids, in which at least a part of the alcohol or of the acid reactant contains a polymerizable unsaturated double bond, are among the preferred thermosetting resins.

As examples of polyhydric alcohols or phenols which can be used to prepare the resins, there may be mentioned: ethylene glycol, propylene glycol, diethylene glycol, tripropylene glycol, triethylene glycol, 1,3-butanediol, neopentyl glycol, and bis-phenol A.

Suitable polybasic acids are: phthalic anhydride, isophthalic acid, terephthalic acid, succinic acid, glutaric acid, adipic acid, sebacic acid, trimellitic acid, pyromellitic acid, hexachloroendomethylenetetrahydrophthalic acid, and tetrachlorophthalic anhydride, benzene dicarboxylic acids being particularly preferred.

The unsaturated carboxylic acids, which are usually employed to modify the polyesters and which may be blended with the aforementioned polybasic acids are dicarboxylic acids and include maleic acid, maleic anhydride, fumaric acid, itaconic acid, citraconic acid, and the like.

The unsaturated polyesters prepared from the aforementioned acids and alcohols are mixed with a polymerizable unsaturated cross-linking agent, for instance, styrene, vinyl toluene or vinyl pyrrolidone, and polymerization is then induced by the addition of a free radical initiator (catalyst) and of an accelerator to the mixture. The actual blending and proportioning of the reactants and reaction promoters may be carried out in any suitable manner.

Among the various thermosetting resins, those derived by cross-linking (for instance, using styrene) unsaturated polyester resins which have been prepared by reacting with a dihydric alcohol (a glycol) a phthalic acid, or an anhydride thereof in admixture with an unsaturated carboxylic acid, such as maleic, are particularly suitable for the preparation of the laminated paving structures of the present invention.

Polyester resins derived from isophthalic acid and containing an unsaturated double bond which has been provided by substituting a portion of the isophthalic acid by an unsaturated acid, such as maleic anhydride, are preferred for the preparation of overlays in accordance with the invention. These resins and their preparation have been described in the prior art. They are non-toxic, cure well between about 40 and about 150° F. and possess a viscosity which permits spraying and mixing them readily at ambient temperatures. On setting, they form a strong durable covering, impervious to solvents and provide excellent protection to the underlying pavement against cracking, water seepage and deterioration, if applied as a part of a laminated structure according to the invention.

A number of overlays were prepared and applied on existing pavements, in accordance with the technique described hereinbefore, and then tested under severe traffic conditions.

In one test series of such overlay applications near a busy boulevard intersection, the asphalt layer was produced by applying it at a rate of 0.4 gallon per square yard on an asphalt concrete pavement. Altogether, six "rumble strips" were placed in succession on the asphalt concrete portion of the road followed by two "rumble strips" on the adjacent Portland cement concrete bridge deck. Finally, one anti-skid strip was placed at the heavily

traveled intersection, in which last case the asphalt rate was 0.25 gallon per square yard. At this intersection, the average traffic volume was 900 motor vehicles daily. In all instances, the resin was applied at the rate of 0.20 gallon per square yard. The size of each overlay was 25 feet in length placed at 50 to 100 feet intervals. The asphalt was 85-100 penetration asphalt applied hot. The resin was an isophthalic acid unsaturated polyester resin prepared by reacting a diethylene glycoethylene glycol mixture (in a 4:1 mol ratio) with a mixture of isophthalic-fumaric acids (in a 3:4 mol ratio). The cross-linking agent was styrene (40% by weight). The rates of application of asphalt, resin, coarse aggregate and sand were as described hereinabove.

The resin, upon being cured, was characterized as follows:

|                                    |        |
|------------------------------------|--------|
| Barcol hardness                    | 33-36  |
| Flexural strength, p.s.i.          | 18,000 |
| Impact strength in ft.-lb./in.     | 6-8    |
| Heat distortion temperature in °F. | 174    |

After two months of service, all of the aforementioned seven overlay strips were found to be in excellent condition and showed no loss of stone ("raveling"), and no cracking of the underlying pavement. On approaching the "rumble strips," the background noise level by the driver's ear, in a car with the windows closed, on the original uncoated (without overlay) pavement was measured to be 94 decibels. As the car crossed each strip, the noise level increased to an average of 104 decibels for a fraction of a second. This heightening of the noise level together with the vibration of the steering wheel was repeated and perceived each time a "rumble strip" was traversed before coming to the intersection, thus giving a clearly perceptible tactile and audible warning to the driver. In addition, even though many drivers suddenly applied the brakes on approaching the intersection over the rumble strips, the structure of these overlays showed no damage upon inspection.

In another test, an anti-skid overlay was applied on an asphalt concrete pavement on a heavily traveled truck road in a petroleum refinery. The asphalt layer which served as a slip plane in this overlay structure was applied as a cationic asphalt-in-water emulsion (200-300 penetration asphalt), after sweeping the pavement. Stone chips (3/8" size) were laid into this asphalt emulsion layer, and the emulsion left to become thoroughly dehydrated. This application was followed by a "choke layer" of a finer aggregate (sand) to cover the asphalt, and the excess of sand was swept off. Thereupon, the same isophthalic acid polyester resin as that described in the preceding series of tests was applied on the "sand choke" and the protruding tips of the coarser aggregate chips. This resin application was followed by another application of resin and then by a final surfacing treatment with sand.

After six months of heavy truck traffic, the overlay was found to be in excellent condition. There are no signs of cracking either in the resin surface of the overlay or in the adjacent surface of the original asphalt concrete pavement.

Finally, in an extensive series of tests, a number of "rumble strips" and "anti-skid" overlays were placed on a wide, heavily used automobile and truck thoroughfare. In applying these overlays, one-half of the road pavement surface (two lanes leading north) was divided into three longitudinal strips, and the asphalt was applied to each at a different application rate. For rumble strips, the overlay section nearest the curb received an asphalt coating at a rate of 0.25 gal. per sq. yd. The center section received 0.4 gal. of asphalt per sq. yd., and the third section ending at the center line of the highway received 0.25 gal. per sq. yd. For anti-skid strips, the corresponding rates of asphalt were 0.15, 0.25 and 0.15 gal. per sq.

yd. In this way, cars traveling in the two northbound lanes had their wheels on each side traversing a surface coating laid on a different thickness of the asphalt slip plane layer. Hot asphalt of 85-100 penetration was employed in forming the slip plane layer.

The asphalt-coated sections of the pavement were embedded with different aggregates. In "rumble strips," three kinds of aggregates were used, ranging from about 3/8" to about 1" in average size as the first course; next, a "choke layer" of a finer aggregate (e.g., No. 8 mesh sand); and, finally, a fine sand layer for surfacing at the top. For anti-skid strips, the coarse aggregate to be embedded in the asphalt consisted of stone chips from about 1/4" to about 3/4" in size, the "choke layer" consisted of No. 8 grits, and the same material was employed to top the surface.

Four different formulations of polyester resins were employed:

- 20 A—A reaction product of diethylene glycoethylene glycol (4:1 mol ratio) and isophthalic-fumaric acids (3:4 mol ratio);  
 B—A reaction product of propylene glycol and isophthalic-maleic acids (1:1 mol ratio);  
 C—A polyester resin similar to that described under (A) with phthalic anhydride being substituted for isophthalic acid;  
 D—A polyester resin similar to that described under (B) with phthalic anhydride again being substituted for isophthalic acid.

Formulations (A) and (B) were blended with 40% styrene, while formulations (C) and (D) were blended with 30% styrene, as the cross-linking agent.

In all instances, methyl ethyl ketone peroxide was employed as the catalyst and cobalt naphthenate as the accelerator for the reaction.

In this particular test series a trailer-mounted traveling spray bar with two spray guns was employed to apply the polyester resin. First, the polyester and the accelerator and the polyester and the catalyst were manually proportioned and blended into two separate mixtures, and each mixture was then fed through a separate line to the spray gun. One gun sprayed the resin blended with the accelerator, and the other sprayed the resin blended with the catalyst, and the two streams met on the pavement surface. Concentration of the catalyst and the accelerator was so adjusted as to give a setting time of about 30 minutes.

Altogether, 12 transverse sections were prepared with the aggregate embedded in the asphalt slip-plane atop the original asphalt concrete (AC) pavement. From 4 to 6 different applications of the four resin formulations, previously described, were applied to these transverse sections, using different application rates. In several applications, calcium carbonate filler was dispersed in proportions varying from 20 to 60% in the resin. In certain controlled sections of the pavement, no resin was employed for the construction of the overlay.

60 After two months, all the overlays on the road surface subjected to testing were examined. All of these overlay structures constructed in accordance with the invention, namely, comprising the asphalt slip layer and the resin coating, were found to be in a satisfactory condition. No cracks could be observed in the underlying original pavement. In test strips laid without the application of polyester resin cover, stones were lost from the asphalt bed, irrespective of the rate employed in applying the asphalt. No loss of stone was noted in the resin-coated overlays.

The following tabulation offers an idea of the extensiveness of the test series described hereinabove. In this table, the first column indicates the kind of resin formulation used (if any); the second column specifies the rate

at which the resin formulation has been applied in gallons per square yard of the surface; and the third column gives the number of test sections (overlays).

Table I

| Resin                      | Application Rate (Gal./ Sq. Yd.) | No. of Test Sections |
|----------------------------|----------------------------------|----------------------|
| None                       |                                  |                      |
| A                          | 0.14                             | 4                    |
| A                          | 0.15                             | 5                    |
| A                          | 0.16                             | 2                    |
| A                          | 0.22                             | 2                    |
| A                          | 0.24                             | 2                    |
| A                          | 0.30                             | 9                    |
| A                          | 0.32                             | 1                    |
| A                          | 0.49                             | 1                    |
| A                          | 0.50                             | 3                    |
| A (20% CaCO <sub>3</sub> ) | 0.30                             | 1                    |
| A (40% CaCO <sub>3</sub> ) | 0.15                             | 1                    |
| A (40% CaCO <sub>3</sub> ) | 0.30                             | 1                    |
| A (60% CaCO <sub>3</sub> ) | 0.15                             | 1                    |
| A (60% CaCO <sub>3</sub> ) | 0.25                             | 3                    |
| A (60% CaCO <sub>3</sub> ) | 0.30                             | 1                    |
| B                          | 0.15                             | 1                    |
| B                          | 0.30                             | 1                    |
| B (40% CaCO <sub>3</sub> ) | 0.18                             | 1                    |
| B (60% CaCO <sub>3</sub> ) | 0.14                             | 1                    |
| B (60% CaCO <sub>3</sub> ) | 0.29                             | 1                    |
| C                          | 0.16                             | 1                    |
| C                          | 0.28                             | 1                    |
| C (40% CaCO <sub>3</sub> ) | 0.14                             | 1                    |
| C (60% CaCO <sub>3</sub> ) | 0.15                             | 1                    |
| C (60% CaCO <sub>3</sub> ) | 0.28                             | 1                    |
| D                          | 0.16                             | 1                    |
| D                          | 0.32                             | 1                    |
| D (40% CaCO <sub>3</sub> ) | 0.14                             | 1                    |
| D (60% CaCO <sub>3</sub> ) | 0.30                             | 1                    |

From the foregoing description of the invention and of the representative results of a number of tests in actual road service, it is clearly apparent that a new and improved composite overlay paving structure is provided by the invention. The structure is not only resistant to water, petroleum and other solvents but, in addition, and contrary to the experience of the prior art and practice, eliminates the tendency towards cracking in the pavement surface underlying such overlays. Because of their high tensile strength, these overlay structures are particularly applicable for the construction and reinforcement of flexible pavements subjected to high traffic loads and wear.

Specifically, the application of these overlays in the construction of "rumble strips," owing to the sawtooth nature of the surface of these strips, facilitates water drainage and reduces the wiping action imposed on the automobile tire treads in wet weather.

Furthermore, these laminated structures, when employed as lightweight overlays, reduce the dead load of the paving structure and enable minimizing of grade changes, while providing a durable surface coating of the pavement surface. Because of the exceptional strength of the hardened thermosetting resin surface, particularly when using isophthalic acid resins, the overlays prepared therewith appear to be exceedingly suitable for use in airstrips for jet aircraft, where jet blasts are known to cause rapid deterioration of the conventional surfaces of air strips.

The paving structures suitable for use in "armor-coats," "rumble strips," and "anti-skid" overlays in accordance with the present invention may be constructed directly on the job by known paving techniques.

However, where the magnitude of the construction job and/or other circumstances do warrant, one need not resort to a large-scale work of paving or resurfacing by applying a "slip-plane" of bituminous material on the pavement base, following it by a layer of coarse stone aggregate, then by a "choke" layer of a finer stone aggregate, and finally by a layer of a thermosetting resin.

Slabs of the paving structure of a suitable specified thickness and size may be prepared (precast) instead at a manufacturing plant and transported to the job to be placed and fitted as needed in the particular area to be paved.

The present application is a continuation-in-part of application Serial No. 73,813, filed by the same applicant on December 5, 1960, now abandoned.

I claim:

1. The process for preparing a paving structure, which comprises applying a layer of a thermoplastic bituminous material onto a rigid base; partially embedding a layer of coarse stone aggregate into said layer of bituminous thermoplastic material; introducing into the interstices of said coarse stone aggregate layer a finer stone aggregate, so that the coarse stone aggregate and the finer stone aggregate together cover completely the surface of the layer of bituminous material; binding the exposed portion of said coarse stone aggregate and the finer stone aggregate layer with a layer of a thermosetting resin; and topping said resin with a layer of a fine particulate solid material.
2. The process as defined in claim 1 wherein said bituminous material is an asphalt.
- 25 3. A process as defined in claim 1 wherein said bituminous material is a tar.
4. The process as defined in claim 1, in which said thermosetting resin is an unsaturated polyester resin.
5. A process as defined in claim 1 wherein said thermosetting resin is a benzene dicarboxylic acid-unsaturated carboxylic acid polyester resin.
- 30 6. A process as defined in claim 1 wherein said thermosetting resin is an isophthalic acid-unsaturated carboxylic acid polyester resin.
- 35 7. A paving structure comprising:
  - (a) a rigid base;
  - (b) a slip-plane layer of a bituminous thermoplastic material upon said base;
  - (c) embedded therein a layer of coarse stone aggregate;
  - (d) a finer stone aggregate covering the surface of the layer of bituminous material and leaving exposed the top portion of the coarse stone aggregate, so that the coarse stone aggregate and the finer stone aggregate together cover completely the surface of the layer of bituminous material;
  - (e) a layer of a thermosetting resin upon said finer stone aggregate and said exposed coarse stone aggregate, said resin penetrating and binding said finer aggregate into a cement-like surface and firmly adhering to the portion of the coarse stone aggregate protruding above said surface; and
  - (f) a top layer of sand adhering to said resin layer.
- 50 8. A paving structure as defined in claim 7 wherein said bituminous material is an asphalt.
9. A paving structure as defined in claim 7 wherein said bituminous material is a tar.
10. A paving structure as defined in claim 7 wherein said thermosetting resin is an unsaturated polyester resin.
- 60 11. A paving structure as defined in claim 7 wherein said resin is an aromatic acid-unsaturated carboxylic acid polyester resin.
12. A paving structure as defined in claim 7 wherein said resin is a benzene dicarboxylic acid-unsaturated carboxylic acid polyester resin.
- 65 13. A rumble-strip paving structure comprising a rigid base, a slip-plane layer of asphalt upon said base, embedded in said layer of asphalt a layer of coarse stone aggregate ranging in size from 1½" to ¾", a layer of a finer stone aggregate to cover the surface of the asphalt and to leave exposed the top portion of the coarse stone aggregate, so that the coarse stone aggregate and the finer stone aggregate together cover completely the surface of the asphalt layer, a layer of a thermosetting resin upon

11

said finer stone aggregate and said exposed portion of the coarse stone aggregate to bind the finer aggregate into a cement-like surface and to adhere firmly to the portion of the coarse stone aggregate protruding above said surface, and a top layer of a fine particulate solid material adhering to the resin layer.

5

12

14. A rumble-strip paving structure as defined in claim 13, wherein said finer stone aggregate covering the asphalt surface with the coarse stone aggregate embedded therein is sand, and the fine particulate solid material atop the resin layer is also sand.

No references cited.